

Sept. 28, 1965

G. J. DODGE

3,208,876

COMBINED INTEGRAL PLASTIC PICTURE FRAME AND MAT

Filed April 24, 1961



1

3,208,876

## COMBINED INTEGRAL PLASTIC PICTURE FRAME AND MAT

George J. Dodge, Westport, N.Y., assignor to Dipak Mfg. Company, Inc., a corporation of New York  
 Filed Apr. 24, 1961, Ser. No. 104,934  
 3 Claims. (Cl. 117—138.8)

This invention relates to an integral picture frame and mat and more particularly to such an article composed of expanded plastic material.

It has long been recognized that proper presentation of art work requires that the art work should be bordered or framed to set it off from its surroundings. Such frames usually are more expensive than the canvas or mat on which the artist paints. Moreover, these frames are commonly made of wood, which is difficult to pack, ship and store since frames will often split and crack due to changing atmospheric conditions. Due to these latent disadvantages, artists often refrain from purchasing frames until their work is completed. However, the artist is placed in a difficult position because he cannot properly visualize how his art work will look in a frame and, therefore, he will often have to modify his work after framing. The above difficulties can be overcome by my invention.

An object of my invention is to provide an integral picture frame and mat which is sturdy, lightweight and economical.

Another object of my invention is to provide a combination picture frame and mat made from expanded plastic, which may be molded to any desired size and shape.

A further object of my invention is to provide an integral picture frame and mat wherein the artist will have his painting framed at all times.

Other and further objects of the invention will be apparent from the following detailed description thereof taken in conjunction with the drawings, in which—

FIG. 1 is a perspective view of my integral picture frame and mat; and

FIG. 2 is a vertical section along line 2—2 of FIG. 1.

As shown in FIGS. 1 and 2, the integral picture frame and mat, generally referred to as 1, comprises a flat work-receiving portion 2, surrounded by a raised frame portion 3, which is coated with my improved composition 4. The outer frame 3 may be of any size or shape and may simulate various grained woods or ceramic designs.

The integral picture frame and mat is obtained by molding a mass of expanded plastic, preferably polystyrene. Foamed or expanded products so produced have, as illustrated in FIG. 2, an internal structure composed of a multitude of closed cells. The outer surface is a thin skin having a smooth pebble-like surface which is the result of the fusion of the closed cells during the molding process. This thin skin is impervious to paints and most liquids. However, many paints contain organic solvents which will cause the skin to dissolve and blend into the paint. Although this solubilizing will allow the paint to adhere to the thin outer skin, it also will destroy the color of the paint as well as the outer surface of the thin skin. Moreover, paints that do not contain organic solvents which will attack the polystyrene cannot adhere to the pebbled surface in a satisfactory manner and an artist attempting to paint on such a surface would find that the paint tends to creep vertically along the surface and spreads to settle in the small depressions in the surface.

Thus, it is apparent that the mat or flat work-receiving portion 2 of the product of this invention is not of itself suitable to be painted upon, but I have provided the coating 4, which is quite critical in nature, to alter these undesirable properties. This completely solves the enu-

2

merated problems by filling in the depressions and sealing the pebbled surface from the solubilizing effects of the organic solvents in artists' paints. Furthermore, the filler pigments provide a surface having enough increased total area, i.e. the exposed surface area of all the individual filler particles, to afford sufficient skin friction for maximum adherence of water-soluble paints.

The coating 4 comprises a group of white inorganic pigments in an organic binder which provides a flat white surface which greatly enhances paint adherence and has the necessary "pull" for the artist's brush. By "pull" is meant the drag or cohesion of the paint and brush with the coated surface.

The constituents of the pigment portion of the composition for forming the coating 4 are as follows: titanium dioxide, rutile titanium-calcium pigment, one commercial form being known as "Ti-Cal," a product manufactured and distributed by the Dupont Company, lithopone and a mineral silicate, such as calcium silicate (wollastonite). The above pigments have all proven necessary to achieve the desired paint retention properties and their respective proportions by weight are as follows: titanium dioxide 34% to 36%, titanium calcium 11% to 12%, lithopone 10% to 11%, and calcium silicate 41% to 45%. The binder portion of the composition is the common liquid commercial grade of shellac resin in an organic solvent and should usually constitute from about 48% to 51% by weight of the total liquid coating composition. The shellac solution employed contains about 25% of resin solids and thus the amount of dried organic binder in the final coating 4 will range from about 20% to about 25% by weight.

The particle size of the pigments will determine the available surface area for the artist's paint and normally will be such that the 90% will pass through a 95 to 98 minus 325 mesh screen.

Many experiments have been conducted but no other composition, either as to the pigment portion or binder portion, has been found which possesses to nearly the same degree, the necessary qualities which make it suitable for the present purpose.

My coating can be applied to the smooth pebbled surface of the expanded plastic by any conventional coating process, but spraying is preferred.

The picture frame and mat combination may be produced by several of the known molding processes for foamed polystyrene and related expanded plastics, i.e. the pre-expanded plastic is placed in a lightweight metal and heat is applied to expand the plastic to fill and conform to the shape of mold. The particular process actually employed would be determined by the size and shape of the integral picture frame and mat, as well as the number to be produced.

The following example is set forth as illustrative of but not as limiting the present invention:

### Example

There was prepared a coating composition having the following composition:

|                         | Percent<br>by weight |
|-------------------------|----------------------|
| Pigments                | 49.56                |
| Binder (liquid shellac) | 50.44                |

The pigment portion of this composition was as follows:

| Ingredient:      | Percent<br>by weight |
|------------------|----------------------|
| Titanium dioxide | 36                   |
| Titanium calcium | 12                   |
| Lithopone        | 11                   |
| Calcium silicate | 41                   |

This composition was sprayed onto the mat portion of an integral molded expanded polystyrene frame and mat so that the coating after evaporation of the shellac solvent had a thickness of approximately  $\frac{1}{32}$  of an inch. The resulting surface was smooth and white and was found to possess excellent paint receiving and retention properties.

It will, of course, be apparent that the improved picture frame and mat in its entirety is a lightweight non-breakable article which will facilitate packaging, shipping and storage. The many beneficial qualities of a plastic material are thereby utilized by my invention and its undesirable properties as to paint retention are overcome. Unlike the normal wooden frames, my frame will not crack or split due to changes in humidity and temperature in the storage area.

As to the decorative features of my invention, the possibilities are limitless. Various designs may be molded into the frame portion to simulate wood, leather or tiled surfaces, and by selecting the proper coloring techniques, attractive facsimiles may be obtained.

Another feature resulting from the use of my improved integral plastic picture frame and mat is that the artist may now visualize how his work will look in the frame during all stages of its development. In this manner, the overall study of the effect of his work may be realized and the artist need not "frame" the painting as required by the use of a regular frame and canvas.

As will be realized, my invention readily lends itself to modern mass production methods. The entire unit may be manufactured by mechanical means in a continuous process and be packaged ready for shipment. The particular method most readily adaptable for producing my integral picture frame and mat is to mold the entire unit in a high pressure, heated mold, and then to spray the coating of pigments and organic binder on that surface of the mat which later will be painted.

Many obvious modifications will occur to those skilled in the art and may be made in the present product without departing from the spirit of the invention claimed as follows.

I claim:

1. An artist's mat comprising a molded, flat work re-

ceiving sheet of expanded plastic and a coating comprising 20-25% shellac and 75-80% of a mixture of finely divided titanium dioxide, rutile titanium calcium, lithopone and calcium silicate secured to one surface of said sheet by said shellac binder, the particle size of the finely divided pigments being such that they will substantially pass through a 325 mesh screen.

2. An artist's mat as claimed in claim 1 in which said plastic is polystyrene and the inorganic ingredients of said coating are present in the following proportions by weight:

|                  | Percent  |
|------------------|----------|
| Titanium dioxide | 34 to 36 |
| Titanium calcium | 11 to 12 |
| Lithopone        | 10 to 11 |
| Calcium silicate | 41 to 45 |

3. An artist's mat as claimed in claim 2 in which said coating contains 80% by weight of inorganic ingredients in the following proportions by weight:

|                  | Percent |
|------------------|---------|
| Titanium dioxide | 36      |
| Titanium calcium | 12      |
| Lithopone        | 11      |
| Calcium silicate | 41      |

and 20% by weight of a shellac binder.

#### References Cited by the Examiner

##### UNITED STATES PATENTS

|    |           |       |          |       |         |
|----|-----------|-------|----------|-------|---------|
| 30 | 2,037,038 | 4/36  | Morrison | ----- | 35-66   |
|    | 2,296,596 | 9/42  | Brown    | ----- | 40-154  |
|    | 2,486,971 | 11/49 | Ohlmann  |       |         |
|    | 2,650,909 | 9/53  | Betsch.  |       |         |
| 35 | 2,681,527 | 6/54  | Sundt    | ----- | 55-66 X |
|    | 2,840,487 | 6/58  | Messina  | ----- | 117-10  |
|    | 2,953,469 | 9/60  | Fox      |       |         |
| 40 | 3,057,097 | 10/62 | Douglas  | ----- | 41-24   |

ALEXANDER WYMAN, Primary Examiner.

EDWARD V. BENHAM, JACOB STEINBERG, EARL M. BERGERT, Examiners.